

May 1, 1934.

K. A. MILAR

1,957,179

#### COATING MATERIAL

Filed May 25, 1931



Witness:

William P. Kilroy

By

Joseph Harris  
Karl A. Milar  
Inventor

## UNITED STATES PATENT OFFICE

1,957,179

## COATING MATERIAL

Karl A. Milar, Evanston, Ill.

Application May 25, 1931, Serial No. 539,738

2 Claims. (Cl. 134—51)

This invention relates to improvements in coating material.

Heretofore, difficulty has been experienced in providing suitable protective coatings for metal surfaces such as the side and end walls, under-frames and other parts of railway cars. If ordinary paints are employed, it is generally necessary to apply at least three coats, particularly on any vertical walls where the tendency is for the 10 thin coating material to run down. Some progress has been made in providing what are known as "car cements", which generally embody an asphaltic base and some undissolved free fibrous material such as asbestos fiber. Such cements 15 embodying undissolved fibrous matter possess the advantage of greater thickness or density and hence have required fewer coats. However, such previously known car cements have not been entirely satisfactory because of the difficulty experienced in keeping the same in a proper condition of fluidity under normal temperature ranges in the United States and temperate zone to permit of proper and efficient application to the metal surfaces. As well known, it is customary 20 to apply the protective coatings to the metal car surfaces in car building plants and railroad shops, which are always more or less open to atmosphere so that, particularly in cold weather, heat has generally been employed to 25 condition the cement for application. Prior to my invention, the customary manner of applying such so-called cements has been by means of trowels or stiff brushes, which obviously involves the use of excessive amounts of the material, increases labor cost of application, and 30 even application of the material.

To some extent, efforts have been made to apply car cements having an asphaltic base and fibrous material therein by spraying, but this 40 method also has resulted in other difficulties. The undissolved or free fibers in such cements heretofore employed frequently cause clogging of the usual spray gun and, unless the cement is heated at time of application, the same frequently becomes so thick or solid as to prevent application by spraying and atomizing. If heating 45 of the cementing material is employed, other difficulties arise in actual practice. If the usual class of operators are instructed to heat the car 50 cement, it frequently happens that so much heat will be applied that the cement becomes so thin or fluid as to allow the fibrous content to settle in the barrels or tanks and, also, heating of the cement as commonly carried out at 55 car building plants results in driving off volatile

substances and chemical changes such that, when the cement is allowed to cool during the nights, it is unfit for application thereafter.

One object of my invention is to provide a durable and efficient coating material, such as car cement, particularly adapted for application to metal surfaces and which comprises an asphaltic base and undissolved fibrous matter, which coating material will always be of sufficient fluid or semi-fluid consistency within the normal range of atmospheric temperatures in the temperate zone as to eliminate the necessity of heat at time of application, will retain the fibrous matter properly in suspension and permit of uniform application of the coating material to the surfaces by spraying.

A further object of my invention is to provide a protective coating material having an asphaltic base and containing undissolved fibrous matter in suspension, which material retains its predetermined consistency within the normal range of atmospheric temperatures so that the coating material may be transported and handled without any special precautions as regards temperature, and sprayed and atomized through a spray gun for application to the surfaces.

Other objects of the invention will more clearly appear from the description and claims herein-after following.

In the drawing forming a part of this specification, Figure 1 is a schematic or diagrammatic view, illustrating conventionally suitable apparatus for mixing or compounding my improved coating material. Figure 2 is an elevational view of suitable apparatus for spraying the coating material, and Figure 3 is a sectional view of a spray nozzle suitable for use in spraying my improved coating material.

In carrying out my invention, I provide a coating material which preferably combines a petroleum asphalt such as roofing black asphalt, gilsonite, a saponifiable or oxidizable oil such as blown soya bean oil, preferably both long and short asbestos fiber, a dense, dark pigment such as dry carbon black and volatile oil, such as benzine.

In order that the coating material may be of the proper consistency when applied and permit of the carrying out of my improved method of application, the material is prepared in the following manner. The roofing black asphalt, which is a petroleum asphalt and may be obtained commercially, is first heated until liquefied, whereupon it is then cut with a hydro-carbon volatile thinner, such as benzine, sufficiently so that, upon

cooling to a normal atmospheric temperature condition, the thinned asphalt will remain in a liquid or semi-fluid condition and of such density that it will retain fibrous matter such as asbestos fiber 5 in suspension, as hereinafter described.

The gilsonite, also obtainable as a commercial product, is likewise heated with a small quantity of saponifiable or oxidizable oil until it liquefies and fuses with the oil and is then similarly cut 10 with a volatile oil, such as benzine, so that it also will retain a liquid or semi-fluid consistency when allowed to cool to normal atmospheric temperatures and of sufficient density to maintain the fibrous matter in suspension, as hereinafter described.

The saponifiable or oxidizable oil, such as blown 15 soya bean oil, the volatile oil, such as benzine, and the pigment, such as dry carbon black, are all ordinary commercial products requiring no special treatment and are mixed with the cut asphalt and gilsonite, as hereinafter described. Asbestos fiber is likewise obtainable commercially and in what is known as short and long fibers, quantities of both of which are preferably used in my improved coating material.

The improved coating material is preferably compounded in the following proportions by weight:

|                      | Per cent |
|----------------------|----------|
| 30 Petroleum asphalt | 20-35    |
| Gilsonite            | 8-20     |
| Oxidizable oil       | 7-17     |
| Volatile oil         | 25-40    |
| Fibrous matter       | 10-30    |
| 35 Pigment           | 0-4      |

For average conditions, I have found a most satisfactory coating material comprised of the following proportions by weight, namely:

|                      | Per cent |
|----------------------|----------|
| 40 Petroleum asphalt | 27       |
| Gilsonite            | 12       |
| Blown soya bean oil  | 10       |
| Benzine              | 34       |
| 45 Asbestos fiber    | 16       |
| Dry carbon black     | 1        |

In preparing and compounding the coating material, the petroleum asphalt and gilsonite are first prepared in the manner hereinbefore set forth and are then placed in a mixer, such as indicated conventionally at 10 in the drawing. To the mixture of cut asphalt and gilsonite is then added the rest of the saponifiable or oxidizable oil and pigment, after which is added and thoroughly whipped into the mixture the fibrous matter, all of this mixing being done at ordinary temperatures. From the mixer 10 the batch is then transferred to an agitator, as indicated conventionally at 11 in the drawing, where the mixture is thoroughly agitated also at normal temperatures. After agitating, the mixture is then placed in barrels or other suitable containers 12 for shipment, the mixture, however, after leaving the agitator and before being deposited in barrels, being passed through a screen, indicated conventionally at 13, for the purpose about to be described. In this connection, due to the consistency of the asphalt and gilsonite, prepared as hereinbefore set forth, it will be understood that the fibrous matter, such as asbestos fiber, will be thoroughly and uniformly distributed throughout the batch by the foregoing mixing and agitating steps and will remain in suspension due to the consistency of the material.

75 Asbestos fiber, as ordinarily carried in stock, is

considered or assumed to be dry, but because of its hydroscopic qualities will absorb a certain amount of moisture from the atmosphere, which moisture to a more or less extent is always present even though the asbestos fiber has all the appearance of being dry. The moisture so absorbed by the asbestos fiber results in small lumps or wads of the fiber being formed, which are exceedingly difficult and practically impossible to break up, after once formed, by any mixing or agitating process. Because of the lumps or wads so formed in the asbestos fiber (which remains undissolved and in suspension in the other materials), I pass the mixture through the screen 13 before delivering into the barrels and so design the mesh of the screen 13 that it will strain out or hold back any of said lumps or wads of the asbestos fiber that would be too big to freely pass through the nozzle of the spray gun used in applying the coating material, and hence insure that the coating material or cement, as it is placed in the barrels for shipment, is of such consistency and, particularly, the asbestos fiber in such size particles, that the material may be readily passed through the nozzle of the spray gun and atomized.

After being placed in the barrels or other suitable form of containers, the material will be shipped to the car building plants or railroad shops, no special precautions being necessary to maintain the desired consistency of the material. Where the material is to be applied, the following is a suitable apparatus that may be employed. The material is first placed in a pressure tank, indicated at 14, which may be mounted on wheels 15 to facilitate its movement from one place to another. The material may be entered through opening 16, which will then be closed. Extending down into the tank 14 to near the bottom thereof is a discharge pipe 17, through which the material is delivered, the same being controlled by valve 18, passing through another screen 19 (interposed in the line for the purposes hereinafter described) and thence through flexible pipe 20 to the spray gun 21. A control valve at the nozzle is indicated at 22. Air under pressure is supplied to the pressure tank 14 from any suitable source, as, for instance, the usual air line 23, through coupling 24, to a Y-25, from one branch of which leads a flexible pipe 26 to the tank 14, said pipe line having a control valve 27 included therein. Preferably, between the control valve 27 and the tank 14, is interposed a branch pipe 28 communicating with a gauge 29 and safety valve 30. From the other branch of the Y-25 leads a flexible pipe 31 to the spray gun 21, said pipe having also included therein a control valve 32 adjacent the nozzle.

The spray gun, as shown, preferably comprises a casing 33, having an apertured bushing 34 threaded into the outer end thereof, the aperture 35 being tapered outwardly as shown in Figure 3. The material supply line 20 terminates in a nozzle 36 within the casing 33, said nozzle projecting partially within the tapered aperture 35. The air supply line 31 delivers the air into a chamber 37 within the casing 33 around the nozzle 36 so that, as the material is forced under pressure through the nozzle and through the bushing, the supply of air, also under pressure, will effectively atomize the material as it leaves the gun.

Referring to the screen 19, which is interposed in the delivery line from the pressure tank, the same is provided to catch or hold back any foreign matter that may inadvertently become mixed with the coating material, such as pieces

89

95

99

95

100

105

110

115

120

125

130

135

140

145

150

of wood, it being not unusual for chips from the barrels to become mixed with the material when the barrels are opened.

With my improved coating material, it is obvi-

ous that the same may be shipped and handled at ordinary temperatures; the fiber remains in suspension; no heat is required during application within the normal range of atmospheric temperatures; and, because of the normal liquid or semi-  
10 liquid condition of the material and the elimination of lumps or wads of the asbestos, the material may be economically and easily applied by the spray gun method, thus insuring uniform application with minimum labor costs.

15 The coating material compounded as herein-before described, will dry out with a tough but not brittle film; the body or consistency of the material is such that, when applied, it will not run but will remain where deposited; will not become brittle or friable even under extreme low temperatures nor become runny or tacky under high atmospheric temperatures; and, when dried out or oxidized, the body of the material retains the desirable elasticity and ductility so as to prevent cracking or checking under vibration or bending within reasonable limits of the metal surface to which applied.

Although I have herein described the preferred composition of my improved coating material and

method of compounding the same, nevertheless all changes and modifications are contemplated that come within the scope of the appended claims.

I claim:

1. A coating material compound including the following substances, thoroughly mixed, and in approximately the following proportions by weight, namely: petroleum asphalt 27%; gilsonite 12%; blown bean oil 10%; asbestos fiber 16%; pigment 1%; and benzine 34%, the mixture being of substantially liquid consistency and the fiber remaining in suspension therein within normal atmospheric temperature ranges.

2. A coating material compound including: petroleum asphalt and gilsonite both pre-cut with a volatile hydrocarbon thinner to a substantially liquid consistency within normal atmospheric temperature ranges, the quantity of the petroleum asphalt being materially greater than that of the gilsonite; blown bean oil, the quantity of the latter being less than the quantity of the petroleum asphalt and gilsonite; and asbestos fiber, all the ingredients being thoroughly mixed and the mixture being of substantially liquid consistency and the fiber remaining in suspension therein within normal atmospheric temperature ranges.

KARL A. MILAR.

30

105

35

110

40

115

45

120

50

125

55

130

60

135

65

140

70

145

75

150